# EUROPEAN PATENT SPECIFICATION

(11) **EP 3 045 557 B1**
(45) Date of publication and mention of the grant of the patent: **17.04.2019**
(21) Application number: 14843474.9
(22) Date of filing: 15.08.2014
(51) Int. Cl.: C22C 45/10, C22C 1/02, C22C 16/00, C22C 1/00, B22D 21/02

(54) **ZIRCONIUM-BASED AMORPHOUS ALLOY AND PREPARATION METHOD THEREFOR**
ZIRKONIUMBASIERTE AMORPHE LEGIERUNG UND HERSTELLUNGSVERFAHREN DAFÜR
ALLIAGE AMORPHE À BASE DE ZIRCONE ET SON PROCÉDÉ DE PRÉPARATION

(30) Priority: 10.09.2013 CN 201310410770
(43) Date of publication of application: 20.07.2016
(73) Proprietor: Dongguan Zhian Intellectual Property Service Co., Ltd., Dongguan, Guangdong 523000 (CN)
(72) Inventor: HUANG, Limin, Dong Guan, Guandong 523808 (CN)
(74) Representative: Meyer, Thorsten
(86) International application number: PCT/CN2014/084500
(87) International publication number: WO 2015/035845

(56) References cited:
- WO-A1-2011/047591
- WO-A1-2011/050680
- WO-A1-2013/087022
- CN-A- 102 061 429
- CN-A- 102 061 429
- CN-A- 103 484 800
- KR-B1- 100 701 027
- US-A1- 2003 079 813

## Description

### FIELD OF THE INVENTION

The invention belongs to the field of metal material and metallurgical technology, and relates to an amorphous alloy, more particularly to a zirconium-based amorphous alloy and a method for preparing the same.

### DESCRIPTION OF RELATED ART

Amorphous alloy has the special structure of disorderly long-range and orderly short-range, thereby featuring high intensity, high rigidity, abrasive resistance, corrosion resistance, wide range of elastic limits, high resistivity, brilliant superconductivity, and low magnetic loss. For these reasons, the amorphous alloy is considered as the most promising new structural material, and has a wide application in the fields of machinery, medical treatment, IT electronics, and military, etc.

WO 2011/047591 A1 discloses a zirconium-based amorphous alloy having a general formula of (ZrₓAl_{y}Cu_{z}Ni_{1-x-y-z})_{100-a-b}ScₐY_{b}, wherein x, y, z are atomic percentages, and a and b are atomic molar ratios, 0.45≤x≤0.60, 0.08≤y≤0.12, 0.25≤z≤0.35, 0<a≤5, and 0≤b<0.1. WO 2013/087022 A1 discloses an alloy having a formula of ZrₐCu_{b}Al_{c}M_{d}Nₑ, wherein M is at least one selected from the group consisting of Ni, Fe, Co, Mn, Cr, Ti, Hf, Ta, Nb, and a rare earth element, N is at least one selected from the group consisting of Ca, Mg, and C, 40≤a≤70, 15≤b≤35, 5≤c≤15, 5≤d≤15, 0≤e≤5, and a+b+c+d+e=100.

For the sake of integrity of amorphous structure, conventional preparation methods of amorphous alloy pose high requirements for the purity of the raw material and the production conditions. For instance, purity of raw material is required to be above 99.9% (mass ratio), and the environment is required to have a rather high vacuum degree in the production process, for example 10⁻⁴-10⁻³ Pa under melting atmosphere, because even small amount of oxygen or other impurity could greatly influence the formation of amorphous alloy. After years of research, it is discovered that zirconium-based amorphous alloy is brilliant at amorphous formation, and that the requirements for the purity of raw material and the production conditions could be slightly lowered by controlling the components
in the amorphous alloy. However, normally, in the production process of amorphous alloy, the demanding conditions still increase the production cost, detain the alloy in the lab, and restrict the application of the amorphous alloy. The production of zirconium-based amorphous alloy in a large scale cannot be realized.

### SUMMARY OF THE INVENTION

In view of the above-described problems, it is one objective of the invention to provide a zirconium-based amorphous alloy and a method for preparing the same. By adding at least one element of Y and Sc and at least one element of Si and C and controlling the content proportions thereof, the requirements for the purity of the raw material, the vacuum degree of the melting, the oxygen content in the melting atmosphere, and the cooling rate are greatly decreased, and in the meanwhile, the comprehensive performance and the stability of the zirconium-based amorphous alloy are improved.

To achieve the above objective, in accordance with one embodiment of the invention, there is provided a zirconium-based amorphous alloy, having the following formula: (Zr_{1-x-y}TiₓHf_{y})ₐ(CuₘNiₙ)_{b}Al_{c}M_{d}Nₑ, in which, a, b, c, d, and e represent numbers of atoms, 30≤a≤ 75 15≤b≤60, 5≤c≤35, 0.1≤d≤20, 0.1≤e≤5, and a sum of a, b, c, d, and e is 100; x, y, m, and n represent atomic fractions of Ti, Hf, Cu, and Ni, respectively, and 0≤x≤0.2, 0≤y≤0.05, 0.2≤m/n≤5. M is at least one selected from Y and Sc, and N is Si or a mixture of C and Si. The alloy consists of a crystalline phase and an amorphous phase, the crystalline phase accounts for between 5 and 50 v. % of a total volume of the zirconium-based amorphous alloy, and an amorphous phase accounts for between 50 and 95 v. % of the total volume of the zirconium-based amorphous alloy.

In a class of this embodiment, a, b, c, d, and e represent the numbers of the atoms, 50≤a≤75, 20≤b≤55, 5≤c≤20, 0.1≤d≤10, and 0.1≤e≤2, and the sum of a, b, c, d, and e is 100. x, y, m, and n represent atomic fractions of Ti, Hf, Cu, and Ni, respectively, and 0≤x≤0.15, 0≤y≤0.03, and 0.4≤m/n≤4.5. The crystalline phase accounts for between 10 and 25 v. % of the zirconium-based amorphous alloy, and the amorphous phase accounts for between 75 and 90 v. % of the zirconium-based amorphous alloy.

In accordance with another embodiment of the invention, there is provided a method for preparing the zirconium-based amorphous alloy. The method comprises: melting raw materials of the zirconium-based amorphous alloy in the presence of an inert gas or in vacuum, and then cooling and shaping the raw materials. The raw materials of the zirconium-based amorphous alloy comprise: Zr, Ti, Hf, Cu, Ni, Al, M, and N, and an addition of each component enable the formula of the zirconium-based amorphous alloy to satisfy (Zr_{1-x-y}TiₓHf_{y})ₐ(CuₘNiₙ)_{b}Al_{c}M_{d}Nₑ.

In a class of this embodiment, the inert gas is at least one selected from the group consisting of helium, neon, argon, krypton, xenon, and radon gas, and a purity of the inert gas is higher than or equal to 94 v. %. The vacuum condition is at a pressure of lower than 1000 pascal which is presented by an absolute pressure. A melting temperature is between 1000 and 3000°C. A melting time is between 0.5 and 10 min.

In a class of this embodiment, the vacuum condition is smaller than 100 pascal. The melting temperature is between 1200 and 2700°C. The melting time is between 2 and 5 min.

In a class of this embodiment, the vacuum condition is between 0.1 and 50 pascal.

Advantages of the zirconium-based amorphous alloy and the method for preparing the same according to embodiments of the invention are summarized as follows:
By adjusting the atomic percentage of each component in the zirconium-based amorphous alloy and by adding non-metallic elements Y and Sc thereto, the preparation requirements of the amorphous alloy can be decreased. In addition, under the same comprehensive performance, the original high requirement on the purity of the raw material is greatly decreased, and a certain amount of impurity elements are allowed to exist in the raw materials. Thus, by properly adjusting the proportions of the non-metallic elements, such as Si and C, in the amorphous alloy, the comprehensive performance of the zirconium-based amorphous alloy cannot be affected; on the contrary, the production cost on the raw materials during the industrialized batch production can be reduced.

The preparation method of the invention is able to produce the zirconium-based amorphous alloy having a critical size of larger than 3 mm. The produced zirconium-based amorphous alloy not only possesses excellent mechanical performance, but also imposes low requirement on the purity of the raw material and the content of the impurity elements. Specifically, it permits existence of less than or equal to 5 % (atomic percentage) of metallic impurity elements and less than or equal to 1% (atomic percentage) of non-metallic impurity elements.

### DETAILED DESCRIPTION OF THE EMBODIMENTS

For further illustrating the invention, experiments detailing a zirconium-based amorphous alloy and a method for preparing the same are described below. It should be noted that the following examples are intended to describe and not to limit the invention.

A zirconium-based amorphous alloy provided in the invention is having the following formula: (Zr_{1-x-y}TiₓHf_{y})ₐ(CuₘNiₙ)_{b}Al_{c}M_{d}Nₑ, in which, a, b, c, d, and e represent numbers of atoms, 30≤a≤75, 15≤b≤60, 5≤c≤35, 0.1≤d≤20, 0.1≤e≤5, and a sum of a, b, c, d, and e is 100; x, y, m, and n represent atomic fractions of Ti, Hf, Cu, and Ni, respectively, and 0≤x≤0.2, 0≤y≤0.05, 0.2≤m/n≤5. M is at least one selected from Y and Sc, and N is Si or a mixture of C and Si.

A crystalline phase accounts for between 5 and 50 v. % of a total volume of the zirconium-based amorphous alloy, and an amorphous phase accounts for between 50 and 95 v. % of the total volume of the zirconium-based amorphous alloy.

Preferably, a, b, c, d, and e represent the numbers of the atoms, 50≤a≤75, 20≤b≤55, 5≤c≤20, 0.1≤d≤10, and 0.1≤e≤2, and the sum of a, b, c, d, and e is 100. x, y, m, and n represent atomic fractions of Ti, Hf, Cu, and Ni, respectively, and 0≤x≤0.15, 0≤y≤0.03, and 0.4≤m/n≤4.5.

The crystalline phase accounts for between 10 and 25 v. % of the zirconium-based amorphous alloy, and the amorphous phase accounts for between 75 and 90 v. % of the zirconium-based amorphous alloy.

Since the industrialized production generally adopts the much cheaper intermediate alloy as the raw material, the produced zirconium-based amorphous alloy always contains some metallic impurity elements, such as Mg, Ca, and Co, and several non-metallic impurity elements, such as C, O, N, B, and P. But for the zirconium-based amorphous alloy of the invention, existence of a certain amount of impurity elements will not affect the performance of the produced zirconium-based amorphous alloy. For example, taken a total amount of the zirconium-based amorphous alloy as a criteria, the zirconium-based amorphous alloy is allowed to contain less than or equal to 5% (atomic percentage) of the metallic impurity elements and less than or equal to 1 % (atomic percentage) of the non-metallic impurity elements. When the contents of the impurities are within the above range, the melting and the preparation of the zirconium-based amorphous alloy will not be affected.

When M is at least one selected from Y and Sc, and N is at least one selected from Si and C, the comprehensive performance of the zirconium-based amorphous alloy is much excellent.

The purities of the raw materials of the zirconium-based amorphous alloy are operable as long as it satisfies the common requirements, and preferable purities thereof are high than 98 wt. %.

In the preparation of the zirconium-based amorphous alloy, the proportion between the crystalline phase and the amorphous phase therein can be adjusted by controlling the composition of the zirconium-based amorphous alloy and controlling the condition for the cooling and shaping according to the common method in the technical field. The condition for the cooling and shaping includes: the cooling rate, the pressure, the material of the die, and the thermal conductivity of the die. The cooling rate is one of the important factors to control proportion of the crystalline phase to the amorphous phase of the zirconium-based amorphous alloy, while the pressure, the material of the die, and the thermal conductivity of the die have a relatively wide selection range, and the cooperative selection thereof can satisfy the condition for the cooling and shaping as along as a proper cooling rate is obtained. In the well-known casting forming methods, the volume percentage of the crystalline phase is generally negatively proportional to the cooling rate. According to the invention, the cooling rate can be selected within the common range, such as higher than 10 K/s, and preferable between 10 and 10⁴ K/s.

In the method for preparing the zirconium-based amorphous alloy of the invention, the inert gas is at least one selected from the group consisting of helium, neon, argon, krypton, xenon, and radon gas, and a purity of the inert gas is higher than or equal to 94 v. %.

The vacuum condition is at a pressure of lower than 1000 pascal which is presented by an absolute pressure.

A melting temperature is between 1000 and 3000°C.

A melting time is between 0.5 and 10 min.

Preferably, the melting time is between 2 and 5 min.

A melting device can be the common melting devices, such as the vacuum arc melting furnace, a vacuum induction furnace, or a vacuum resistance furnace.

The zirconium-based amorphous alloy has excellent shaping performance. Thus, the cooling and shaping can adopt the common die-casting methods and the stainless steel and copper alloy materials in the technical filed. The cooling of the die can adopt the water cooling and oil cooling methods.

### Example 1

Raw materials having purities of 99 wt. % for the zirconium-based amorphous alloy were added into a vacuum arc melting furnace, the vacuum arc melting furnace was then deaerated until a pressure therein was 10 pascal. After that, argon gas having a purity of 99.9 v. % was introduced into the vacuum arc melting furnace as a protective gas, and the melting was performed at a temperature of 1500°C for 3 min to make the raw materials for the zirconium-based amorphous alloy fully melted. Components and contents (atomic percentages) of the raw materials for the zirconium-based amorphous alloy were as follows: 50% of Zr, 2% of Ti, 15% of Cu, 10% of Ni, 15% of Al, 4% of Y, 2% of Sc, and 2% of Si.

A melted sample was finally casted into a copper alloy die by a die-casting method for cooling and shaping so as to obtain the zirconium-based amorphous alloy.

### Example 2

Raw materials having purities of 99 wt. % for the zirconium-based amorphous alloy were added into a vacuum arc melting furnace, the vacuum arc melting furnace was then deaerated until a pressure therein was 10⁻¹ pascal. After that, argon gas having a purity of 99.9 v. % was introduced into the vacuum arc melting furnace as a protective gas, and the melting was performed at a temperature of 1650°C for 3 min to make the raw materials for the zirconium-based amorphous alloy fully melted. Components and contents (atomic percentages) of the raw materials for the zirconium-based amorphous alloy were as follows: 60% of Zr, 3% of Ti, 2% of Hf, 12.5% of Cu, 7.5% of Ni, 5% of Al, 5% of Y, 3% of Sc, 1.5% of Si, and 0.5% of C.

A melted sample was finally casted into a copper alloy die by a die-casting method for cooling and shaping so as to obtain the zirconium-based amorphous alloy.

### Example 3

Raw materials having purities of 99 wt. % for the zirconium-based amorphous alloy were added into a vacuum arc melting furnace, the vacuum arc melting furnace was then deaerated until a pressure therein was 10⁻¹ pascal. After that, argon gas having a purity of 99.9 v. % was introduced into the vacuum arc melting furnace as a protective gas, and the melting was performed at a temperature of 1600°C for 3 min to make the raw materials for the zirconium-based amorphous alloy fully melted. Components and contents (atomic percentages) of the raw materials for the zirconium-based amorphous alloy were as follows: 60% of Zr, 1.5% of Ti, 0.5% of Hf, 10.5% of Cu, 9.5% of Ni, 8% of Al, 0.5% of Y, 1.2% of Sc, and 0.3% of Si.

A melted sample was finally casted into a copper alloy die by a die-casting method for cooling and shaping so as to obtain the zirconium-based amorphous alloy.

### Example 4

Raw materials having purities of 98 wt. % for the zirconium-based amorphous alloy were added into a vacuum arc melting furnace, the vacuum arc melting furnace was then deaerated until a pressure therein was 200 pascal. After that, argon gas having a purity of 99 v. % was introduced into the vacuum arc melting furnace as a protective gas, and the melting was performed at a temperature of 1500°C for 3 min to make the raw materials for the zirconium-based amorphous alloy fully melted. Components and contents (atomic percentages) of the raw materials for the zirconium-based amorphous alloy were as follows: 50.5% of Zr, 0.5% of Hf, 30% of Cu, 7.5% of Ni, 10% of Al, 0.8% of Y, and 0.8% of Si.

A melted sample was finally casted into a copper alloy die by a die-casting method for cooling and shaping so as to obtain the zirconium-based amorphous alloy.

### Example 5

Raw materials having purities of 98 wt. % for the zirconium-based amorphous alloy were added into a vacuum arc melting furnace, the vacuum arc melting furnace was then deaerated until a pressure therein was 50 pascal. After that, argon gas having a purity of 99 v. % was introduced into the vacuum arc melting furnace as a protective gas, and the melting was performed at a temperature of 1600°C for 3 min to make the raw materials for the zirconium-based amorphous alloy fully melted. Components and contents (atomic percentages) of the raw materials for the zirconium-based amorphous alloy were as follows: 57.5% of Zr, 2.3% of Ti, 1.2% of Hf, 23% of Cu, 6.3% of Ni, 9.2% of Al, 0.2% of Y, and 0.3% of Si.

A melted sample was finally casted into a copper alloy die by a die-casting method for cooling and shaping so as to obtain the zirconium-based amorphous alloy.

### Comparison example 1

The preparation of the zirconium-based amorphous alloy is the same as that of Example **1** except that the raw materials for the zirconium-based amorphous alloy have purities of 99.8 wt. %.

Raw materials having purities of 99.8 wt. % for the zirconium-based amorphous alloy were added into a vacuum arc melting furnace, the vacuum arc melting furnace was then deaerated until a pressure therein was 10 pascal. After that, argon gas having a purity of 99.9 v. % was introduced into the vacuum arc melting furnace as a protective gas, and the melting was performed at a temperature of 1500°C for 3 min to make the raw materials for the zirconium-based amorphous alloy fully melted. Components and contents (atomic percentages) of the raw materials for the zirconium-based amorphous alloy were as follows: 50.9% of Zr, 29.9% of Cu, 7.4% of Ni, 9.8% of Al, and 2% of Y.

### Comparison example 2

Raw materials having purities of 99.7 wt. % for the zirconium-based amorphous alloy were added into a vacuum arc melting furnace, the vacuum arc melting furnace was then deaerated until a pressure therein was 10 pascal. After that, argon gas having a purity of 99.9 v. % was introduced into the vacuum arc melting furnace as a protective gas, and the melting was performed at a temperature of 1800°C for 3 min to make the raw materials for the zirconium-based amorphous alloy fully melted. Components and contents (atomic percentages) of the raw materials for the zirconium-based amorphous alloy were as follows: 55% of Zr, 2% of Ti, 16.5% of Cu, 13.5% of Ni, 9.6% of Al, 0.4% of Y, and 3% of Nb.

The products were finally detected by metallographic analysis, bending strength test, and oxygen content detection, and detection results are listed in Table **1.**

**Table 1 Parameters of zirconium-based amorphous alloys prepared by Examples 1-5 and comparison examples 1-2**

| | Proportion of crystalline phase (%) | Bending strength (megapascal) | Oxygen content (ppm) |
|---|---|---|---|
| Example **1** | 23 | 1970 | 800 |
| Example **2** | 20 | 1890 | 860 |
| Example **3** | 22 | 1785 | 720 |
| Example **4** | 12 | 2170 | 800 |
| Example **5** | 15 | 2035 | 1000 |
| Comparison example **1** | 7 | 1750 | 1300 |
| Comparison example **2** | 5 | 1600 | 1450 |

It is indicated from Table **1** that according to the components and the contents thereof and the preparation method of the invention, the amorphous alloy that has excellent performance can be acquired under low purity of the raw materials and loosened preparation condition. The amorphous alloy produced in the invention has the proportion of the crystalline phase of between 10 and 25% and the oxygen content of between 600 and 1200 ppm, and has much better mechanical performance compared with the conventional zirconium-based amorphous alloy prepared in the comparison example.

Unless otherwise indicated, the numerical ranges involved in the invention include the end values.

## Claims

1. A zirconium-based alloy, having the following formula:
(Zr_{1-x-y}TiₓHf_{y}),(CuₘNiₙ)_{b}Al_{c}M_{d}Nₑ
wherein 30≤a≤75, 15≤b≤60, 5≤c≤35, 0.1≤d≤20, 0.1≤e≤5, 0≤x≤0.2, 0≤y≤0.05, 0.2≤m/n≤5, a+b+c+d+e = 100, a, b, c, d, and e are atomic numbers, x, y, m, and n are atomic fractions, M is at least one selected from Y and Sc, N is Si or a mixture of C and Si; the alloy consists of a crystalline phase and an amorphous phase, the crystalline phase accounts for between 5 and 50 vol. % of the total volume of the zirconium-based alloy, and the amorphous phase accounts for between 50 and 95 vol. % of the total volume of the zirconium-based alloy.

2. The alloy of claim 1, wherein 30≤a≤75, 20≤b≤55, 5≤c≤20, 0.1≤d≤10, 0.1≤e≤2, a+b+c+d+e = 100, 0≤x≤0.15, 0≤y≤0.03, 0.4≤m/n≤4.5; the crystalline phase accounts for between 10 and 25 vol. % of the zirconium-based alloy, and the amorphous phase accounts for between 75 and 90 v. % of the zirconium-based alloy.

3. A method for preparing the alloy of claim 1, comprising: melting raw materials of the zirconium-based alloy in the presence of an inert gas or in vacuum, and then cooling and shaping the raw materials; wherein:
the inert gas is helium, neon, argon, krypton, xenon, radon gas, or a mixture thereof, and a purity of the inert gas is higher than or equal to 94 vol. %;
the vacuum is lower than 1000 Pa of absolute pressure;
a melting temperature is between 1000 and 3000°C;
a melting time is between 0.5 and 10 min;
the raw materials of the zirconium-based alloy comprise: Zr, Ti, Hf, Cu, Ni, Al, M, and N, and
an addition of each component enable the formula of the zirconium-based alloy to satisfy (Zr_{1-x-y}TiₓHf_{y})ₐ(CuₘNiₙ)_{b}Al_{c}M_{d}Nₑ.

4. The method of claim 3, wherein the vacuum condition is smaller than 100 pascal; the melting temperature is between 1200 and 2700°C; and the melting time is between 2 and 5 min.

5. The method of claim 3, wherein the vacuum is between 0.1 and 50 Pa of absolute pressure.

## Patentansprüche

1. Legierung auf Zirkoniumbasis mit der folgenden Formel:
(Zr₁₋ₓ₋yTiₓHf_{y})ₐ(CuₘNiₙ)_{b}Al_{c}M_{d}Nₑ
wobei 30 ≤ a ≤ 75,
15 ≤ b ≤ 60, 5 ≤ c ≤ 35, 0,1 ≤ d ≤ 20, 0,1 ≤ e ≤5, 0 ≤ x ≤0,2,
0 ≤ y ≤ 0,05, 0,2 ≤ m/n ≤5, a+b+c+d+e = 100, a, b, c, d und e sind Atomzahlen, x, y, m und n sind Atomfraktionen, M ist mindestens ein Element, ausgewählt aus Y und Sc, N ist Si oder eine Mischung aus C und Si; die Legierung besteht aus einer kristallinen Phase und einer amorphen Phase, die kristalline Phase macht zwischen 5 und 50 Vol .-% des Gesamtvolumens der Legierung auf Zirkoniumbasis aus, und die amorphe Phase macht 50 bis 95 Vol.-% der Legierung des Gesamtvolumens der Legierung auf Zirkoniumbasis aus.

2. Legierung nach Anspruch 1, wobei 30 ≤ a ≤ 75, 20 ≤ b ≤ 55, 5 ≤ c ≤ 20, 0,1 ≤ d ≤ 10, 0,1 ≤ e ≤ 2, a+b+c+d+e = 100, 0 ≤ x ≤ 0,15, 0 ≤ y ≤ 0,03, 0,4 ≤m/n ≤4,5; die kristalline Phase macht zwischen 10 und 25 Vol.-% des Gesamtvolumens der Legierung auf Zirkoniumbasis aus, und die amorphe Phase macht 75 bis 90 % der Legierung auf Zirkoniumbasis aus.

3. Verfahren zur Herstellung der Legierung nach Anspruch 1, umfassend: Schmelzen von Ausgangsmaterialien der Legierung auf Zirkoniumbasis in Gegenwart eines Inertgases oder im Vakuum und dann Abkühlen und Formen der Ausgangsmaterialien; worin:
das Inertgas Helium, Neon, Argon, Krypton, Xenon, Radongas oder eine Mischung davon ist und eine Reinheit des Inertgases höher als oder gleich 94 Vol.-% ist;
das Vakuum niedriger als 1000 Pa absoluter Druck ist;
die Schmelztemperatur zwischen 1000 und 3000°C liegt;
die Schmelzzeit zwischen 0,5 und 10 min liegt;
die Ausgangsmaterialien der Legierung auf Zirkoniumbasis umfassen: Zr, Ti, Hf, Cu, Ni, Al, M, und N, und
eine Beimischung von jeder Komponente ermöglicht, dass die Formel der Legierung (Zr_{1-x-y}TiₓHf_{y})ₐ(CuₘNiₙ)_{b}Al_{c}M_{d}Nₑ genügt.

4. Verfahren nach Anspruch 3, wobei der Vakuumzustand kleiner als 100 Pascal ist; die Schmelztemperatur zwischen 1200 und 2700°C liegt; und die Schmelzzeit beträgt zwischen 2 und 5 min.

5. Verfahren nach Anspruch 3, wobei das Vakuum zwischen 0,1 und 50 Pa Absolutdruck beträgt.

## Revendications

1. Alliage à base de zirconium, ayant la formule suivante:
(Zr₁₋ₓ₋yTiₓHf_{y})ₐ(CuₘNiₙ)_{b}Al_{c}M_{d}Nₑ
où 30≤a≤75,
15≤b≤60, 5≤c≤35, 0,1≤d≤20, 0,1≤e≤5, 0≤x≤0,2,
0 ≤ y ≤ 0,05, 0,2 ≤ m/n ≤ 5, a + b + c + d + e = 100, a, b, c, d et e sont des nombres atomiques, x, y, m et n sont des fractions atomiques, M est au moins un élément choisi parmi Y et Sc, N est Si ou un mélange de C et Si; l'alliage est constitué d'une phase cristalline et d'une phase amorphe, la phase cristalline représente entre 5 et 50 % en volume du volume total de l'alliage à base de zirconium et la phase amorphe représente entre 50 et 95 % en volume du volume total de l'alliage à base de zirconium.

2. Alliage selon la revendication 1, dans lequel 30 ≤ a ≤ 75, 20 ≤ b ≤ 55, 5 ≤ c ≤ 20, 0,1 ≤ d ≤ 10, 0,1 ≤ e ≤ 2, a + b + c + d + e = 100, 0 ≤ x ≤ 0,15, 0 ≤ y ≤ 0,03, 0,4 ≤ m/n ≤ 4,5; la phase cristalline représente entre 10 et 25 % en volume de l'alliage à base de zirconium, et la phase amorphe représente entre 75 et 90 % en volume de l'alliage à base de zirconium.

3. Procédé de fabrication de l'alliage selon la revendication 1, comprenant: la fusion de matières premières de l'alliage à base de zirconium en présence d'un gaz inerte ou sous vide, puis le refroidissement et la mise en forme des matières premières; où
le gaz inerte est de l'hélium, du néon, de l'argon, du krypton, du xénon, du radon ou un mélange de ceux-ci, et la pureté du gaz inerte est supérieure ou égale à 94 % en volume;
le vide est inférieur à 1000 Pa de pression absolue;
la température de fusion est comprise entre 1000 et 3000°C;
le temps de fusion est compris entre 0,5 et 10 min;
les matières premières de l'alliage à base de zirconium comprennent: Zr, Ti, Hf, Cu, Ni.Al, M et N, et
une addition de chaque composant permet à la formule de l'alliage à base de zirconium de satisfaire à (Zr_{1-x-y}TiₓHf_{y})ₐ(CuₘNiₙ)_{b}Al_{c}M_{d}Nₑ.

4. Procédé selon la revendication 3, dans lequel la condition de vide est inférieure à 100 Pascals; la température de fusion est comprise entre 1200 et 2700°C; et le temps de fusion est compris entre 2 et 5 min.

5. Procédé selon la revendication 3, dans lequel le vide est compris entre 0,1 et 50 Pa de pression absolue.
